

## UNITED STATES PATENT OFFICE

JEAN GEORGES PENCHE, OF ROUSSILLON, FRANCE, ASSIGNOR, BY MESNE ASSIGNMENTS, TO DU PONT RAYON COMPANY, OF NEW YORK, N. Y., A CORPORATION OF DELAWARE

## PROCESS OF DISCHARGING

No Drawing. Application filed June 25, 1928, Serial No. 288,297, and in Great Britain July 26, 1927.

This invention relates to the treatment of artificial silk having as its base an organic derivative of cellulose (ester or ether) in the form of filaments, threads, yarns and fabrics 5 containing them. More especially, it relates to a process for discharging a dye on threads of artificial silk in the form of skeins, webs or fabrics containing them.

This invention has for an object a process 10 for discharging dyed threads of artificial silk the base of which is a cellulose derivative (ester or ether) without destroying the dynamometrical qualities of the thread or its suppleness to the touch.

15 Another object of this invention is a process for discharging dyed artificial silk threads on predetermined areas, whereby patterns may be formed which, upon dyeing with the original or different dyestuffs, produce superposed shade effects or two-colored effects respectively.

Another object of this invention is a process 20 for simultaneously discharging and dyeing artificial silk having as its base a cellulose derivative (ester or ether).

Other objects will become apparent from the following description and appended claims.

According to this invention, the dyed artificial silk threads or yarns are discharged by 25 means of animal or vegetable charcoal or any other body having high adsorbing properties. These materials may be applied as a suspension in a liquid or in the form of a paste.

I have found that the discharging action takes place more rapidly and completely 30 when it is carried out at a high temperature and when the contact between the fiber and the adsorbing body is very intimate. Furthermore, I have found that the discharging action of the agent may be in certain cases accelerated by causing the fiber to swell either before or during the discharging process by 35 means of any suitable swelling agent.

When the discharging composition is applied in the form of a paste, such as animal charcoal mixed with a thickening agent or filler, the process is carried out by steaming. 40 It is followed by rinsing with cold or tepid

liquid by means of which the paste is removed. Rinsing at a high temperature as long as the animal charcoal is in contact with the fiber or fabric must be avoided for it might cause a discoloration on areas not desired. The fiber or fabric is then washed, finished, dried and further treated in any suitable or desirable manner. A fabric or fiber treated by the discharging method just described retains all of its desirable properties. 55

The present invention is capable of many applications. First, it affords means for completely removing a dye on cellulose acetate threads or threads of other cellulose esters or ethers. This may be of great importance. For instance, in the failure of a certain shade, the dyestuffs may be removed without affecting in any way the dynamometrical qualities of the threads or their suppleness to the touch. 60 65

Instead of completely removing the dye from the entire surface of the material treated, it may be discharged from any local or predetermined areas. By this procedure various patterns, such as white discharge effects on a colored background, may be obtained. Materials which have been locally discharged in this manner can be subsequently treated to produce ornamental effects by dyeing with a dye similar to the original dyestuff used or with a new dyestuff. When a fabric having locally or predetermined discharged areas is treated with the same coloring matter with which it was originally dyed, superposed shade effects will be obtained. 70 75 80 85

The regions or areas which have not been subjected to this discharging process will be darker than the regions which have been subjected to the discharging process. If a different dyestuff is used from the original dyestuff, two-colored effects will be obtained. A repetition of the same sequences of operation will produce fabrics having motley effects. 90 95

By regulating the composition of the paste and regulating also the temperature of the operation and its duration, it is possible to obtain more or less complete discharging effects. It is thus possible by printing the same 100

fabric with different pastes, i. e. different ingredients and/or different proportions of the same ingredients, to obtain discharges of different or varying intensity.

5 The invention also contemplates a simultaneous discharging operation and re-dyeing of the discolored material. To obtain this result it suffices to add to the paste containing the discharging substance compounds capable of performing the re-dyeing. For example, a basic coloring matter and a body capable of fixing it on the cellulose acetate fibers, such as sodium resorcinate, may be mixed with the paste. A direct coloring matter susceptible of dyeing cellulose acetate and of a different shade from that of the background of the fabric may also be added to the paste containing the adsorbing body if a two-tone effect fabric is desired.

10 20 A saponifying agent may even be added to the paste whereby the cellulose acetate fibers are superficially saponified. If desired, together with this saponifying agent a coloring agent or compound adapted to dye the cellulose may be mixed with the paste whereby the material treated will be dyed. Discharges of different or varying intensities may also be secured by treating predetermined areas of threads of organic derivatives 15 of cellulose or fabrics containing the same with a composition including an adsorbing agent and a swelling agent and treating other predetermined areas with a composition in which there is no swelling agent.

25 30 35 40 45 50 55 60 65 70 75 80 85 90 95 100 105 110 115 120 125 130

In the case of fabrics containing fibers of artificial silk and certain other or foreign fibers, such as natural silk, a discharge effect may be obtained upon said foreign fibers without the addition of other substances. However, a suitable quantity of the discharging agents usually employed for said foreign fibers may be mixed with the paste which contains only the adsorbing agent, whereby the said usual discharging agent will act more particularly with respect to the other fibers. The charcoal or other adsorbing agent in this process will act more particularly with respect to the artificial silk fibers.

In all applications of the present invention where a printing paste is made use of, all the ingredients which are usually employed in the industry may be mixed with said paste containing the charcoal. For example, various thickening agents, such as gum arabic, gelose, dextrin, etc., may be added. I have found that such products as kaolin, fuller's earth or infusorial earth give satisfactory results when used in the paste. Kaolin gives especially good results, and compositions including it produce well-defined discharge effects rapidly. There may be mixed with the paste such products as glucose or glycerin which enable the paste to retain a certain binding action after the

drying operation which takes place immediately after printing.

The dyes for cellulose acetate available to the dyer or printer on which discharge effects may be obtained, according to this invention, have an extremely extensive range of colors.

The present process may be applied to artificial silks comprising exclusively cellulose esters or ethers. It is also applicable to materials containing these cellulose derivatives and fillers or adjuvants. It is as effective with bright as with dull silks.

In order to more clearly explain the invention, the following specific examples are given:

*Example I.*—A veil of cellulose acetate thread dyed with 1. methylaminoanthraquinone (Duranol red G British Dyestuffs Corporation) is printed with a paste formed with

|                 | Grams |
|-----------------|-------|
| Animal charcoal | 20    |
| Gum tragacanth  | 75    |
| Water           | 1,000 |

The tissue is then steamed for one hour at 95° C. The veil rinsed cold, washed and dried exhibits perfectly white discharge effects at the places treated.

*Example II.*—A satin with a cellulose acetate weft is dyed with 1.4 diaminoanthraquinone (Duranol violet 2R.) and is printed on the satin side with a paste containing

|                 | Grams |
|-----------------|-------|
| Dimethylaniline | 30    |
| Animal charcoal | 15    |
| Gelose          | 80    |
| Water           | 1,000 |
| Glycerin (28°)  | 50    |

It is then steamed for half an hour. After washing, the printed places are discharged in white. The same result may be obtained on the same satin tissue when it has received a dulling treatment before the application of the discharge process.

*Example III.*—A cellulose acetate tissue with linen cloth cording dyed with an azo dye derived from aniline or its derivatives and dihydroxyquinoline (Dispersol yellow 3G) is printed after dyeing with a paste containing

|                         | Grams |
|-------------------------|-------|
| Animal charcoal         | 20    |
| Arabic gum              | 500   |
| Water                   | 500   |
| Ammonium sulpho cyanide | 50    |

It is steamed for half an hour with dry steam, then rinsed and dyed again with the same dye. A tissue is obtained in this manner with superposed shade effects. The same tissue after the local discharge treatment is dyed in a Celatine blue bath. The portions which are not discolored dye green and the discharged portions dye blue.

*Example IV.*—A tissue with a cellulose

acetate web and a natural silk crepe weft is prepared and dyed green with, on the one hand, diaminoanthraquinone (Acetoquinone blue—Etablissement Kuhlmann) and 1, amio-  
5 noanthraquinone (Acetoquinone yellow Etablissement Kuhlmann) for the acetate and, on the other hand, with Malachite green, Colour Index No. 657, for the natural silk. The tissue is printed with a paste containing

|                                       | Grams |
|---------------------------------------|-------|
| Animal charcoal                       | 20    |
| Senegal gum                           | 500   |
| Water                                 | 500   |
| Glycerin                              | 50    |
| 15 Rhodamine S. Colour Index No. 743. | 80    |
| Sodium resorcinate                    | 10    |

and dried. After steaming for three-quarters of an hour, rinsing and drying, a tissue is obtained having a red printed pattern on a green background.

*Example V.*—A veil made of cellulose acetate thread dyed with diaminoanthraquinone (Duranol blue) is printed with a paste comprising

|                        |            |
|------------------------|------------|
| Animal charcoal        | 5 grams    |
| Ammonium sulphocyanate | 5 grams    |
| Kaolin                 | 5 grams    |
| Glycerin               | 5 ccm.     |
| 30 Water               | 30-50 ccm. |

The paste is dried and the fabric is then steamed for half an hour at 105° C. After washing, the printed portions are discharged in very pure white.

Naturally, any number of printing rollers can be used, each one coated with a paste of different composition and obtain in this manner a polychrome impression as complex as may be desired.

It is well understood that the invention is not restricted to the examples given but that it includes all the discharge or discoloring effects obtained by the application of extremely divided adsorbing agents, whatever may be the treatment to which the fiber, yarn or tissue has been submitted or to which it will be submitted after discharge.

I claim:

50 1. A process for discharging dyed fabrics containing threads of an organic derivative of cellulose which comprises treating said fabrics with a composition containing charcoal.

55 2. A process for discharging dyed fabrics containing threads of an organic derivative of cellulose which comprises treating said fabrics with a composition containing animal charcoal.

60 3. A process for discharging dyed fabrics containing threads of cellulose acetate which comprises treating said fabrics with a composition containing charcoal.

65 4. A process for discharging dyed fabrics containing threads of cellulose acetate which

comprises treating said fabrics with a composition containing animal charcoal.

5. A process for discharging dyed fabrics containing threads made of cellulose acetate which comprises treating said fabrics with a 70 composition containing charcoal and a swelling agent for the cellulose acetate.

6. A process for discharging dyed fabrics containing threads of an organic derivative of cellulose which comprises applying a composition 75 containing charcoal and a swelling agent to certain predetermined areas, applying a composition containing charcoal without a swelling agent to other predetermined areas whereby discharge effects of varying 80 intensities are obtained.

7. A process for discharging dyed fabrics containing threads of cellulose acetate which comprises applying a composition containing charcoal and a swelling agent to certain 85 predetermined areas, applying a composition containing charcoal without a swelling agent to other predetermined areas whereby discharge effects of varying intensities are obtained.

8. A process for discharging dyed fabrics containing threads of an organic derivative of cellulose which comprises treating said fabrics with a composition containing charcoal and steaming.

9. A process of discharging dyed fabrics containing threads of an organic derivative of cellulose which comprises subjecting said fabrics to the joint action of a swelling agent and charcoal and then steaming.

10. A process of treating dyed fabrics containing threads of an organic derivative of cellulose which comprises applying a composition containing charcoal, a swelling agent and a coloring agent and then steaming.

In testimony whereof, I have affixed my signature to this specification.

JEAN GEORGES PENCHE.